

## UNITED STATES PATENT OFFICE

ERNEST J. PIEPER, OF LANCASTER, PENNSYLVANIA, DILLON F. SMITH, OF PENSACOLA, FLORIDA, AND CLARENCE C. VOGT, OF LANCASTER, PENNSYLVANIA, ASSIGNEES TO ARMSTRONG CORK COMPANY, OF LANCASTER, PENNSYLVANIA, A CORPORATION OF PENNSYLVANIA

## DISTRIBUTING BINDER OVER FIBROUS MATERIALS

No Drawing. Continuation of application Serial No. 236,359, filed November 28, 1927. This application filed August 2, 1930. Serial No. 472,752.

The present invention relates to a process of distributing a binder over fibrous materials and to the article produced thereby, and more especially to a process wherein the 5 binder is distributed uniformly and in a desired minimum amount to the surface of the fibers. The process is particularly applicable to the distribution of a binder over fibrous materials which are afterward 10 formed or molded into fibrous articles.

Various methods of coating the fibers of fibrous materials have been employed or suggested. These processes have included saturating a dry mass of the fibrous material with a liquid binder or a solid binder in liquid solution and evaporating the solvent. In such processes, a considerable amount of binder is required to coat the fibers. Moreover, the fibers, because of their dry porous 15 condition, tend to absorb the binder and its solvent as well, further increasing the amount of binder and solvent necessary. It has also been proposed to apply binding material to the fibers in the form of an emulsion. This requires the formation of an 20 emulsion with the presence of emulsifying agents which may be objectionable in the completed article and have to be removed during the process. It has also been suggested 25 that materials such as sand, clay or fibrous materials be first wetted with water and stirred into a plastic mass of asphalt to form paving material. The resultant 30 mass has been in the nature of a plastic paving composition. It has also been suggested 35 that solid resins be finely divided and mixed with pulp, which is afterwards heated.

We have found that a binding material can be economically and uniformly distributed 40 over the fibers of a fibrous mass with the desired minimum coating of the binder on the fibers, by forming a fluid pulp of the fibrous material and adding to it and mixing in the binding material thinned 45 with a solvent to sufficient fluidity to form thin liquid films by adsorption onto the surfaces of the fibers. Neither emulsification of the binding material nor heat is required to effect the distribution of the binding material 50 over the fibers. The distribution of

the binder over the fiber surfaces can be carried out at ordinary room temperatures simply by heating or stirring the solution of the binding material into the fluid pulp. The solution of the binding material should 55 be sufficiently fluid at normal temperatures so as to distribute itself by adsorption in a thin film over the surfaces of the fibers. The binding material and its solvent should be such as to be nonsoluble or difficultly soluble 60 in the liquid which forms the fluid pulp suspension. The fluid pulp is in the nature of a suspension in the fluid, usually water, of the fibrous material, the proportion of the water to the fibrous material being large, as 65 distinguished from the mere wetting or soaking of a fibrous mass with water.

The pulp should be of sufficient fluidity so that when it is beaten or otherwise agitated, the solution of the binding material can be 70 readily broken up into droplets which are dispersed throughout the fluid pulp. We have found that the fluidity of the pulp is important in getting a thorough dissemination and distribution of a minimum amount 75 of binder in the form of thin films uniformly applied to the fibers throughout the mass. The pulp is in the form of a suspension in the liquid as distinguished from being merely wetted or soaked by the liquid. 80

The following is a specific example of our process:

A fluid pulp such as a paper pulp or a pulp for making a fiber-board is formed having an excess of water to render the pulp 85 sufficiently fluid to be handled by the usual pumping machinery for handling pulps. The large excess of water is also necessary in order to get uniform distribution and application of the desired minimum amount 90 of binder to the fibers. The amount of fiber to water is not over about 5 to 10%, although usually less than 5% of fiber to water is employed.

A pulp of this character can be readily 95 handled in the usual pulp machinery. After the fluid pulp has been formed, the binder is added to it and thoroughly stirred into the fluid pulp at normal room temperatures and without heating. In the case of making 100

a fiber-board, a binder of equal parts of asphaltum and stearine pitch is preferably employed. The asphaltum and stearine pitch are substantially non-soluble in water.

- 5 The asphaltum and stearine pitch are brought into a liquid condition with a solvent which is also substantially non-soluble in water, such as petroleum naphtha, which can be later evaporated. Usually an amount 10 of naphtha about equal in weight to the asphaltum and stearine pitch is used. This solution of asphaltum and stearine pitch to an amount of about 10% of the weight of the dry pulp is added to the suspended pulp 15 and is thoroughly stirred or beaten into the pulp until the binder is uniformly distributed over the pulp fibers. The fibers have been previously saturated with the water so that the binder is apparently applied to the 20 surfaces of the fibers, as distinguished from the absorption of the binder and solvent into the fibers which would take place if the fibers were dry.

The liquid binder solution does not have 25 to be emulsified or finely divided, but can be simply dumped into the beater or other stirring device containing the pulp and the stirring carried out to disseminate the binder over the fibers with a uniformity comparable to that obtained when adding the binder in a fine water emulsion. The large amount of water in proportion to the fiber and to the binder serves to cause the even distribution of the binder over the fibers 30 held in suspension in the liquid pulp.

The process is economical in that no emulsifying agents are needed and the solution of the binding material can be simply dumped into the beater and beaten into the 40 cold liquid pulp.

During the beating of the fluid pulp, the body of the binding material solution which is dumped in is broken up into droplets which are readily dispersed and disseminated throughout the mass of pulp because of its fluid condition, and since the droplets are non-miscible in the water, they are adsorbed onto the surface of the fibers. The presence of the fiber in the pulp suspension 45 probably contributes to the breaking up and dispersion of the liquid into small separated droplets. The beating of the pulp forms a fluid droplet suspension of the relatively small amount of liquid binder which is non-miscible with the water, and the binder, while in such fluid suspension, is uniformly distributed and adsorbed in a liquid condition onto the surfaces of the fibers, giving a distribution comparable to that obtained 50 with the use of emulsions, but without the presence of objectionable emulsifying agents or the steps of preparing the emulsion.

After the binder has been stirred into and distributed through the fluid pulp, the pulp 55 may be run through suitable forming ma-

chines, such as pulp-board machines, to form sheets which may be dried and are then ready for use. In the case of such articles as pulp or fiber-boards, a relatively small amount of binder is required, and the 70 above process allows such binder to be uniformly distributed and applied as surface coatings to the fibers to cause the desired adherence of the fibers in the completed board with a minimum of binder. 75

The invention, however, is not limited to making pulp or suspensions of fibrous materials which are to be used for making paper, pulp-board or fiber-board. It can be utilized to great advantage in making an insulation 80 board, which is light and porous. It can also be used to distribute the binder in greater amounts to make fibrous objects which are to be dense or waterproof, or which are to be molded or highly compressed, either with or without heating. 85

In all cases, the amount of the distributing liquid, such as the water, is large compared with that of the fibrous material and the binder, since the excess of the distributing 90 medium, such as water, is requisite to produce the desired even distribution of the binder over the fibers. The process is therefore applicable to fibrous materials, in general, including paper pulp and other fibrous 95 pulps made from various materials.

While water is the preferred distributing medium in making the liquid pulp or fibrous suspension, other distributing mediums might be employed, such as alcohol or other liquids which do not act as solvents for the binder employed. 100

While bituminous binding materials such as asphalts and pitches dissolved in suitable volatile solvents are the binders usually employed in making fiber-boards, other binders may be used which are brought into a sufficiently fluid condition by a suitable solvent. Oils, such as linseed oil, may be thinned by suitable solvents and distributed over the fibers by this process. As examples of other binders may be cited the nitrocellulose materials dissolved on nitrocellulose solvents, varnishes dissolved on various varnish solvents, wax tailings dissolved in petroleum naphthas, etc. In any case, the solution of the binder material as added should be sufficiently fluid so as to form thin uniform films by adsorption onto the 105 surfaces of the fibers. 110

The present application is a continuation of our earlier copending application Serial No. 236,359, filed November 28, 1927.

While we have specifically described the 125 preferred embodiments of our invention, it is to be understood that the invention is not so limited, but may be otherwise embodied and practiced within the scope of the following claims: 130

We claim:

1. The process of distributing binding material in liquid form through a fibrous material, which comprises forming a fluid suspension of the fibrous material and a binding material and a solvent therefor, in a suspending liquid in which the binder and the solvent are substantially non-soluble, and stirring the suspension to distribute the liquid solution of the binder on the fibers.

2. The process of distributing binding material in liquid form through a fibrous material, which comprises forming a fluid suspension of the fibrous material and a binding material thinned with a solvent to sufficient fluidity to form thin liquid films by adsorption onto the surfaces of the fibers in a suspending liquid in which the binder and its solvent are substantially non-soluble, and stirring the suspension so as to distribute the binder in liquid form over the fibers.

3. The process of distributing binding material in liquid form through a fibrous material, which comprises forming a fluid suspension of the fibrous material and a binding material thinned with a solvent to sufficient fluidity at normal temperatures to form thin liquid films by adsorption onto the surfaces of the fibers in a suspending liquid in which the binder and its solvent are substantially non-soluble, and stirring the suspension so as to distribute the binder in liquid form over the fibers.

4. The process of distributing binding material in liquid form through a fibrous material, which comprises forming a water suspension containing not over about 10% of the fibrous material and also a binding material thinned with a solvent of sufficient fluidity to form thin liquid films by adsorption onto the surfaces of the fibers, both the binding material and its solvent being substantially nonsoluble in water, and stirring the water suspension so as to distribute the binder in liquid form over the fibers.

5. The process of distributing a bituminous binding material in liquid form through a fibrous material, which comprises forming a water suspension of the fibrous material and the bituminous binding material thinned with a solvent substantially non-soluble in water to sufficient fluidity to form thin liquid films by adsorption onto the surfaces of the fibers, and stirring the water suspension so as to distribute the bituminous binder in liquid form over the fibers.

6. The process of distributing a bituminous binding material in liquid form through a fibrous material, which comprises forming a water suspension of the fibrous material and a bituminous binding material thinned with naphtha to a sufficient fluidity to form thin liquid films by adsorption onto the surfaces of the fibers, and stirring the

water suspension so as to distribute the bituminous binder in liquid form over the fibers.

In testimony whereof we have hereunto set our hands.

ERNEST J. PIEPER.  
DILLON F. SMITH.  
CLARENCE C. VOGT.

70

75

80

85

90

95

100

105

110

115

120

125

130